

# United States Patent Office

2,940,932

Patented June 14, 1960

1

2,940,932

## LUBRICANTS CONTAINING STABILIZED DISPERSIONS OF FATTY ACID SALTS

Arnold J. Morway, Clark, N.J., assignor to Esso Research and Engineering Company, a corporation of Delaware

No Drawing. Filed Oct. 1, 1957, Ser. No. 687,366

8 Claims. (Cl. 252—40.5)

This invention relates to lubricating oil compositions. Particularly, it relates to lubricating fluids and semi-fluids containing metal salt of low molecular weight fatty acid and a synthetic ester.

Alkaline earth metal salts of  $C_2$  to  $C_4$  fatty acids, particularly calcium acetate, have been recently recognized as extremely effective lubricating oil additives for reducing wear and imparting extreme pressure characteristics to the lubricant. In the past, these salts have been suspended in oil by means of simple metal soap, or by complexing the  $C_2$  to  $C_4$  fatty acid salts with higher molecular weight fatty acid salts or soaps, or by forming oil-water emulsions containing the  $C_2$  to  $C_4$  fatty acid salts. However, for some applications, these prior methods are not wholly satisfactory. Thus, the presence of higher molecular weight salts or soaps result in high deposit formation when the lubricant is used as a crank-case lubricant, while the emulsion type materials are rather corrosive because of their water content and are also somewhat unstable, tending to separate upon storage. It has also been proposed to dehydrate the emulsion type of material, but while this reduces the danger of corrosion, it still results in an unstable product and unless the dehydration is carefully controlled a grainy unsatisfactory dispersion is obtained.

It has now been found that metal salts of low molecular weight fatty acids may be stably dispersed in the presence of a synthetic ester. In this manner, simple lubricating dispersions can be formed which have excellent extreme pressure properties and good load-carrying characteristics.

The metal salts operable in the invention will include alkaline earth metal salts such as calcium, barium, strontium, etc. of low molecular weight  $C_2$ — $C_4$  fatty acids such as acetic acid, propionic acid and butyric acid. Specific examples of these salts will include calcium acetate, calcium butyrate, barium acetate and barium propionate.

The synthetic esters used to stably disperse the salt are those esters consisting of aliphatic saturated hydrocarbon chains interlinked by one or two ester linkages and containing a total of about 15 to 40, e.g. 20 to 35, carbon atoms. Such esters will include simple esters and diesters prepared from  $C_6$  to  $C_{20}$  alkanols or  $C_2$  to  $C_6$  glycols with either  $C_6$  to  $C_{12}$  alkanoic acids or  $C_6$  to  $C_{12}$  alkanedioic acids. Preferred esters are those prepared from alkanedioic acids and Oxo alcohols. The Oxo alcohols are isomeric mixtures of branched chain primary alkanols produced by the reaction of an olefin with hydrogen and carbon monoxide in the presence of a cobalt catalyst to form a mixture of aldehydes, which aldehydes are then hydrogenated to form the Oxo alcohol. Such Oxo alcohols and their preparation are well known in the art.

Specific examples of esters of the above types will include diesters such as: di-( $C_{10}$  Oxo) adipate; di(2-ethylhexyl) sebacate; di-( $C_8$  Oxo) sebacate; 1,6-hexamethylene glycol di-(2-ethylhexanoate); 1,10-decamethylene glycol di-(caprylate); and simple esters such as: nonyl heptanoate; decyl laurate; octadecyl laurate; decyl stearate; etc.

2

The base oil of the lubricating composition may be either a mineral lubricating oil, a synthetic lubricating oil or both. Synthetic oils include: mono- and di-esters prepared from alkanols or glycols with mono- or dicarboxylic acids such as are described above; complex esters, e.g. the complex ester formed by reacting one mole of sebacic acid with two moles of tetraethylene glycol and two moles of 2-ethylhexanoic acid; esters of phosphoric acid; halocarbon oils; polyglycols; silicone oils; etc.

5 10 Particularly desirable synthetic oils are the silicone polymer oils having lubricating oil viscosity, i.e. viscosities of about 25 to 3500 SSU at 100° F. These oils have the general formula:



wherein R is a hydrocarbon radical, which may be halogen (e.g. chlorine) substituted or unsubstituted and including alkyl, aryl, haloaryl, alkylaryl, arylalkyl and cycloalkyl radicals containing between about 1 to 8 carbon atoms per radical. Specific examples of such oils include phenylmethylsilicone, dimethylsilicone and chloro-phenylmethylsilicone. These materials are known in the art and are available under trade-names such as DC (Dow Corning) F-258 Silicone Fluid, DC F-60 Silicone Fluid and DC 550 Silicone Fluid. A preferred silicone oil is Dow Corning 710 Silicone Fluid, which is a phenylmethylsilicone polymer oil having a viscosity at 25° C. of 500 centistokes.

20 25 30 35 40 Various additive materials can also be added to the lubricating composition in amounts of about 0.1 to 10.0 weight percent, based on the total weight of the composition. Examples of such additives are: detergents such as calcium petroleum sulfonate; oxidation inhibitors such as phenyl-alphanaphthylamine; viscosity index improvers such as polyisobutylene; corrosion inhibitors such as sorbitan monoleate; pour depressants; dyes; and the like.

45 50 55 The compositions of the invention will therefore comprise lubricating oil, a wear reducing amount of the metal salt and at least a sufficient amount of synthetic ester to maintain said salt in a stable dispersion. In terms of weight percent, such compositions will usually comprise about 5 to 40 wt. percent of salt and about 2 to 50 wt. percent synthetic ester, the remainder being lubricating oil.

55 60 65 The compositions of the invention are best prepared by forming the metal salt in situ in an inert menstruum to thereby obtain a fine dispersion. This is done by neutralizing the fatty acid with a metal base (i.e. hydroxide or oxide) in the presence of the synthetic ester, followed by heating to temperatures of about 300 to 500° F. e.g. 300 to 400° F. in order to dehydrate the mixture. Lubricating oil, other than the synthetic ester, may also be present during the neutralization. Although the proportions of acid, base, ester and lubricating oil may be such as to form a finished lubricant, it is preferred to first make a concentrate and then to dilute the concentrate with additional lubricating oil to form the finished lubricant. To insure a completely homogeneous final lubricant, the lubricant may be homogenized in a Gaulin homogenizer, a Morehouse mill, a Charlotte mill, etc.

65 70 The invention will be further understood by the following examples which include preferred embodiments of the invention:

### Example I

(A) 10 weight percent of di-( $C_{10}$  Oxo) adipate (the  $C_{10}$  Oxo alcohol was prepared from tripropylene) and 40 weight percent of a mineral lubricating oil of 80 SUS at 210° F., were charged to a fire heated kettle. 17

weight percent of hydrated lime was added and an intimate smooth, uniform slurry was formed. 25 weight percent of glacial acetic acid was next added, and the temperature rose to 210° F. due to the heat of reaction. External heating was applied and the mixture was heated to about 310° F. for about one hour until the product was completely dehydrated. The product was then allowed to cool to about 200° F. and was then passed through a Charlotte mill to form a smooth product having a semi-fluid consistency.

(B) For comparison purposes, a lubricant containing dehydrated calcium acetate was prepared in the manner of I(A) above, except that 50 weight percent of mineral lubricating oil was used and no ester oil was present.

The products of (A) and (B) above were each tested for stability as follows: A quart sample bottle was filled with the lubricant and stored in an oven maintained at 210° F. for five days, after which the sample was examined for salt precipitation. The product of (A),

25 weight percent of the product of Example V was

intimately mixed with 75 weight percent of a mineral

lubricating oil having a viscosity of 80 SUS at 40° F.

This mixture was then passed through a Gaulin homo-

genizer operating at 6000 p.s.i. shear.

#### Example VI

20 weight percent of the base material of Example 10 V was intimately mixed with 80 weight percent of Dow Corning Fluid 710 (a phenylmethylsilicone polymer having a viscosity at 250° C. of 500 cs.). The mixture was then homogenized in a Gaulin homogenizer at 6000 p.s.i. shear.

All of the products of the preceding examples were smoothly homogeneous compositions. The compositions in terms of initial ingredients, and the properties of the preceding examples of the invention are summarized in the following table:

| Composition (Wt. Percent)                        | Examples   |       |       |       |            |       |       |
|--------------------------------------------------|------------|-------|-------|-------|------------|-------|-------|
|                                                  | I(A)       | II    | III   | IV    | V          | VI    | VII   |
| Glacial acetic acid.....                         | 25.0       | 7.5   | 7.5   | 7.5   | 25.0       | 6.25  | 5.00  |
| Hydrated lime.....                               | 17.0       | 5.1   | 5.1   | 5.1   | 16.75      | 4.19  | 3.35  |
| Di-(C <sub>10</sub> Oxo) adipate.....            | 10.0       | 3.0   | 3.0   | 3.0   | 58.25      | 14.56 | 11.65 |
| Mineral lubricating oil (80 SUS at 210° F.)..... | 48.0       | 84.4  | 70.0  | 14.4  | 75.00      | ----- | 80.00 |
| Phenylmethylsilicone oil.....                    | -----      | ----- | 70.0  | ----- | -----      | ----- | ----- |
| Chlorinated phenylmethylsilicone oil.....        | -----      | ----- | ----- | 70.0  | -----      | ----- | ----- |
| Properties:                                      |            |       |       |       |            |       |       |
| Consistency.....                                 | semi-fluid | fluid | fluid | fluid | semi-fluid | fluid | fluid |
| Viscosity (SSU) —                                |            |       |       |       |            |       |       |
| 100° F.....                                      | 1,795      | 1,664 | ----- | ----- | 1,795      | ----- | ----- |
| 210° F.....                                      | 139        | 199   | ----- | ----- | 136        | ----- | ----- |
| 4-Ball Wear Test (1,800 r.p.m.—10 Kg.—           | 0.32       | 0.32  | 0.40  | 0.40  | -----      | 0.30  | 0.30  |
| 1 hour—75° C.) mm. dia. scar.....                |            |       |       |       |            |       |       |

which contained the synthetic ester, showed no salt precipitation. The product of (B), which contained no ester, showed about a one-eighth inch layer of precipitated salt on the bottom of the sample bottle. It is thus seen that the presence of the ester stabilizes the salt dispersion.

#### Example II

30 weight percent of the final dehydrated product of Example I(A) was intimately mixed with 70 weight percent of a mineral lubricating oil having a viscosity of about 80 SUS at 210° F. This mixture was then passed through a Gaulin homogenizer operating at 6000 p.s.i. shear.

#### Example III

A lubricant was prepared in a manner similar to that of Example II except that 70 weight percent of Dow Corning Silicone Fluid 710 was used in place of the 70 weight per cent mineral oil.

#### Example IV

Example III was repeated except that General Electric 81406 Silicone Fluid was used in place of the Dow Corning Fluid. The G.E. silicone was a chlorinated phenylmethyl silicone.

#### Example V

16.75 weight percent of hydrated lime and 58.25 weight percent of a di-(C<sub>10</sub> Oxo) adipate (the C<sub>10</sub> Oxo alcohol was prepared from tripropylene) were charged to a steam-heated kettle and mixed to a smooth slurry. 25 weight percent of glacial acetic acid was slowly added while stirring and the temperature rose to 230° F. where large quantities of steam were evolved. The mixture was further heated to about 320° F. to completely dehydrate the calcium acetate. This base material was then cooled to about 200° F. at which point it was homogenized in a Gaulin homogenizer operating at 6000 p.s.i. shear, and then allowed to cool to room temperature.

40 As seen from the preceding table, lubricants prepared by dispersing anhydrous calcium acetate in the presence of a synthetic ester formed stable lubricants which had very low wear characteristics. Examples I(A) shows that semi-fluids may be prepared in this manner, while Examples II, III and IV illustrate the formation of fluid type lubricants prepared by further diluting the concentrate of Example I(A) with various lubricating oils.

45 For comparison purposes, a blend was prepared consisting of the di-(C<sub>10</sub> Oxo) adipate, mineral lubricating oil and phenylmethylsilicone oil in the same proportions as in Example III, but which contained no calcium acetate. This blend gave a wear scar dia. of 2.85 mm. in the 4-ball wear test, while the composition of Example IV which was a similar composition except that it also contained calcium acetate gave a wear scar diameter of 0.40 mm. This illustrates the effectiveness of the fatty acid salt in reducing wear. The product of Example IV was also tested for storage stability and showed no sign of oil separation or salt precipitation when stored for four weeks at 80° F.

50 Example V illustrates a semi-fluid lubricant in which the synthetic ester also served as the sole lubricating oil, while Examples VI and VII again illustrate fluid materials formed by further dilution of the concentrate of Example V with other lubricating oils.

55 In summary, this invention relates to lubricants containing an anhydrous alkaline earth metal salt of a C<sub>2</sub> to C<sub>4</sub> fatty acid which is stabilized against salt precipitation by a synthetic ester. Generally at least about 25 wt. percent of the ester, based on the weight of salt should be present. In cases where the ester is also a lubricating oil in its own right, then compositions can be prepared consisting only of the anhydrous salt and the ester. Although the working examples thus far presented are only of anhydrous calcium acetate and a di-ester, other salts and esters contemplated by the invention can also be readily prepared in the same manner. For example, a composition can be prepared consisting

of 10.0 wt. percent anhydrous barium propionate, 15 wt. percent of n-octyl stearate and 75 wt. percent of mineral lubricating oil of 80 SUS viscosity at 210° F.

It is thus seen that excellent stable lubricants may be prepared containing synthetic ester and the metal salt of the C<sub>2</sub> to C<sub>4</sub> fatty acid as the sole metal salt component, i.e. without the necessity of having present higher molecular weight salts, e.g. calcium stearate or calcium petroleum sulfonate.

What is claimed is:

1. A lubricating oil composition consisting essentially of a lubricating oil, about 5 to 40 wt. percent of anhydrous alkaline earth metal salt of C<sub>2</sub> to C<sub>4</sub> fatty acid and about 2 to 50 wt. percent of a synthetic ester consisting of saturated aliphatic hydrocarbon chains joined by two ester linkages and containing a total of 15 to 40 carbon atoms.

2. A composition according to claim 1, wherein said synthetic ester is also a lubricating oil.

3. A composition according to claim 1, wherein said salt is calcium acetate.

4. A lubricating oil composition according to claim 1, wherein said lubricating oil is a mineral lubricating oil.

5. A lubricating oil composition according to claim 1, wherein said ester is a diester of a dicarboxylic acid and an alkanol.

6. A composition according to claim 1, wherein said salt is calcium acetate.

7. A process for preparing a lubricating oil composition which comprises neutralizing an alkaline earth metal base with a C<sub>2</sub> to C<sub>4</sub> fatty acid in a synthetic ester lubricating oil consisting of saturated aliphatic hydrocarbon chains joined by two ester linkages and containing a total of 15 to 40 carbon atoms, dehydrating said synthetic ester lubricating oil containing said neutralized metal base at temperatures of 300° to 400° F., to form a lubricating oil composition containing an anhydrous salt, followed by mixing until smooth.

8. The process according to claim 7, wherein said alkaline earth metal base is neutralized with said acid in a mixture of mineral lubricating oil and said synthetic ester.

15

References Cited in the file of this patent

UNITED STATES PATENTS

|           |                          |               |
|-----------|--------------------------|---------------|
| 2,079,051 | Sullivan et al. -----    | May 4, 1937   |
| 2,467,147 | Morway et al. -----      | Apr. 12, 1949 |
| 2,581,127 | Morway et al. -----      | Jan. 1, 1952  |
| 2,607,735 | Sproule et al. -----     | Aug. 19, 1952 |
| 2,692,233 | Cottle -----             | Oct. 19, 1954 |
| 2,744,870 | Stillebroer et al. ----- | May 8, 1956   |
| 2,820,815 | Matuszak et al. -----    | Jan. 21, 1958 |

FOREIGN PATENTS

744,685      Great Britain ----- Feb. 15, 1956